

(No Model.)

J. COFFIN.

PROCESS OF CONTINUOUSLY ANNEALING AND PLATING WIRE.

No. 399,382.

Patented Mar. 12, 1889.



WITNESSES.

James Cranston  
Chas W. Hoffman

John Coffin, INVENTOR.

# UNITED STATES PATENT OFFICE.

JOHN COFFIN, OF JOHNSTOWN, PENNSYLVANIA, ASSIGNOR TO THE  
CAMBRIA IRON COMPANY, OF PENNSYLVANIA.

## PROCESS OF CONTINUOUSLY ANNEALING AND PLATING WIRE.

SPECIFICATION forming part of Letters Patent No. 399,382, dated March 12, 1889.

Application filed July 28, 1888. Serial No. 281,264. (No model.)

*To all whom it may concern:*

Be it known that I, JOHN COFFIN, a citizen of the United States, residing at Johnstown, in the county of Cambria and State of Pennsylvania, have invented certain new and useful Improvements in the Process of Continuously Annealing and Plating Wire; and I do hereby declare the following to be a full, clear, and exact description of the invention, such as will enable others skilled in the art to which it appertains to make and use the same.

My invention relates to the art of continuously annealing wire and coating it with a metallic coating, commonly called "galvanizing," but more properly "plating."

In the process of continuous annealing and plating it has been customary to first pass the wire through an annealing-bath of red-hot lead and then through an acid bath, and then through the zinc. The object of the acid bath is to thoroughly cleanse the surface of the wire from oxide. There would be great gain accomplished if the wire could be passed from the lead annealing-bath directly to the zinc-coating bath without passing through an intermediate bath of acid, because where an acid bath is used the wire has to be cooled almost cold to prevent the acid from being vaporized, and then the cold wire in passing into the plating-bath chills the body of the bath, so that the operation is delayed. If the plating-bath were not chilled at all, the operation would be somewhat delayed, because the wire has to come to the temperature of the fusing-point of the plating-metal before any plating will take place. It has been heretofore impossible to dispense with the acid bath between the annealing and the plating baths, because where the wire is exposed to the atmospheric action a film of oxide is deposited on the wire, which prevents the adhesion of the plating-metal. To overcome this objection and make it possible to run directly from the annealing-bath to the plating-bath is the feature of my present invention.

To carry my invention into effect, I first pass the wire through an acid bath to remove all traces of dirt and oxide, thence through a red-hot-lead annealing-bath. I then carry it through a suitable conduit filled with reducing-gas to the plating-bath, thence through

the plating-bath, and finally wipe from it the surplus metal and coil it upon reels in the usual manner.

My invention, then, consists, in the main part, in the reversal of the order of the acid and annealing baths and the gas-filled conduit, which makes this reversal possible.

The object of my invention is to cheapen the process of annealing and plating by preventing a waste of acid from vaporization, and to make possible a more rapid progression of the wire through the baths, as the time in the plating-bath is the usual limit to the speed of manipulation; and by bringing the wire into the plating-bath at or near the temperature 65 of the metal contained therein very little time is required in this bath.

The conduit which forms part of my invention is similar in construction to one which I describe in an application, Serial No. 281,263, for a patent for process of annealing and plating wire, filed simultaneously with this application. It is desirable to make this conduit of suitable length, so that the wire will slowly cool from the temperature of the lead annealing-bath to about the temperature of the plating-bath before reaching it, for if the conduit were so short that the wire reached the plating-bath at a full red heat there would be some 80 hardening and stiffening of the wire, due to the sudden cooling from the full red to the temperature of the plating-bath, and the object of annealing would be somewhat thwarted. To get sufficient length without occupying too 85 much floor-space, I make the conduit of A shape, and place in the apex of the A a suitable roller to conduct the wires over, it being understood in this, as in other plating processes, that it is desirable to carry many wires 90 through the several baths simultaneously. To prevent gas from escaping from the conduit and to prevent the atmosphere from entering it, I seal the ends of the conduit by immersing them in the baths. Thus one leg of the 95 conduit is fixed entirely under the surface of the lead annealing-bath, and the other leg of the conduit is fixed entirely under the surface of the plating-bath. If no provision were made to prevent it, the contained gas in the conduit 100 would become very hot from the many wires passing through it, and the temperature of

the wire would not be reduced enough before reaching the metal of the plating-bath. To keep the gas cool in the conduit, I cool the outside of the conduit by spraying on it jets of water from pipes near the apex of the A. The water flows down the sloping sides, and is carried away by means of stop-gutters located at the bottoms of the legs and above the surfaces of the baths. I supply gas to the conduit through a suitable pipe. There is no wastage of gas, except through some trifling leakage, therefore a large supply of gas is not required, and the small amount of gas I use is thoroughly dry. I prefer to use hydrogen, carbonic-oxide, or other suitable reducing-gas, and thoroughly dry it by causing it to bubble through sulphuric acid, for it is well known that a wet gas, which may be reducing at a high temperature, will be oxidizing at a low temperature.

Referring to the annexed plate of drawings, which forms part of this specification, Figure 1 is a sectional elevation; Fig. 2, a plan of my invention, and Fig. 3 a detail on line X Y of Fig. 1.

Like letters of reference refer to like parts throughout.

W represents a wire in course of passage through the several baths, the arrows showing its direction of passage.

B represents the acid bath, A the lead annealing-bath, and C the plating-bath.

a, b, and c represent suitable sinkers in the several baths, to retain the wire under the surface of the contained liquid.

a' is a roller located at the end of the acid bath B, the office of which is to guide the wires into the bath.

b' is a roller located between the baths B and A, the office of which is to guide the wires in their passage between these baths.

D represents the conduit. This conduit, as is shown by drawings, is A shape, and has located at its apex the roller d', which serves as a guide to the wires through the conduit.

The roller d' is entirely within the conduit, but may have one of its journals extend through a stuffing-box, so as to have power applied from without to revolve the roller d' and assist in the passage of the wires. One end of the conduit dips under the surface of the lead bath A and the other end dips under the surface of the plating-bath C, the object of this seal being to prevent the egress of gas or ingress of air.

d<sup>2</sup> is a pipe to supply the conduit with dry gas.

d<sup>3</sup> d<sup>3</sup> are spray-pipes to spray water on the outside of conduit D, to keep its surface cool. d<sup>4</sup> d<sup>4</sup> are stop-gutters attached to the legs of the conduit above the surfaces of the baths, to conduct away the water which has been sprayed upon the outside of the conduit and which has run down its sloping sides.

The overflow of the stop-gutters d<sup>4</sup> d<sup>4</sup> is shown at d<sup>5</sup> d<sup>5</sup>.

The conduit D is rectangular in section, so

as to accomodate many wires. The form is clearly shown in Fig. 3, which is a section on line X Y of Fig. 1.

The dots in Fig. 3 represent the wires within the conduit, one of which is marked W.

In operating my invention at least one wire is always kept within the conduit. To introduce other wires, the end of the wire to be introduced is fastened to the wire which is already in the conduit, when its passage through will introduce the new wire. In the course of operation, should a wire become broken in the conduit, a new wire is introduced by fastening its end to any of the progressing wires. The roller d' at the top of the conduit is not grooved to separate the wires, but is a plain roller, so that if the wires do not maintain their relative position of entering the conduit no trouble is experienced.

I have spoken of my invention as a process of plating wire. I do not confine myself narrowly to the commercial article known as "wire," but wish to have my invention embrace all metallic strips, woven webbing, twisted strands, linked wire, or other articles which it is usual to plate and which ordinarily are long enough to be treated by the continuous method.

By my invention I am not restricted to a particular kind of acid, as the office of the acid bath which I use is merely to clean the wire. Thus I may use a bath of dilute sulphuric acid, after which I might place a bath of running water to remove the adhering acid. It would be permissible to use sulphuric acid in my process, because the heat of the annealing-bath would be sufficient to drive off the hydrogen which otherwise would be objectionable; or I might use a bath of any other acid or any combination of baths, or might use some other annealing-bath, or might substitute for the annealing-bath a tubular furnace; and I may use any proper plating-metal.

Having fully described my invention, what I claim as new, and desire to secure by Letters Patent, is—

1. The process of annealing and plating wire by continuous operation, consisting in passing the wire, first, through a suitable cleaning-bath of acid; second, through an annealing-bath of red-hot lead or other medium; third, through a sealed conduit filled with reducing-gas, and, fourth, through a bath of molten zinc or other suitable plating-metal, substantially as and for the purpose set forth.

2. The process of annealing and plating wire by continuous operation, consisting in passing the wire through an annealing-bath, thence directly through a conduit filled with reducing-gas, and thence through a bath of plating-metal, substantially as and for the purpose set forth.

In testimony whereof I affix my signature in presence of two witnesses.

Witnesses: JOHN COFFIN,  
HARRY A. SHIELDS,  
JAMES CRANSTON.